

## UNITED STATES PATENT OFFICE

2,501,992

## LUBRICATING OILS

James O. Clayton, Berkeley, Calif., and William H. Alderson, Bahrein Island, Arabia, assignors to California Research Corporation, San Francisco, Calif., a corporation of Delaware

No Drawing. Application October 28, 1948,  
Serial No. 706,084

8 Claims. (Cl. 252—42.7)

1

This invention relates to hydrocarbon lubricating oils and the like containing a new and useful combination of additive materials. More particularly, it relates to mineral lubricating oil containing a new and useful combination of phenate and selenide additives.

It is an object of the invention to provide a new and useful combination of additive materials to be incorporated in hydrocarbon lubricating oil and the like to accomplish a higher level of improvement than provided by additive materials and combinations thereof heretofore in use.

It is a further object of the invention to produce hydrocarbon lubricating oil and the like having in higher degree than heretofore, the following characteristics: high detergency, that is, the property of maintaining pistons, piston rings and piston ring slots in internal combustion engines in a clean condition; resistance to oxidation; and a low degree of corrosion of alloy bearings, such as, cadmium-silver and copper-lead bearings.

These and other objects of the invention will be apparent from the following description and the appended claims.

In accordance with the invention, there is incorporated in an oil of lubricating viscosity a small amount each of a salt of a phenol containing an ether substituent on the aromatic nucleus and an aliphatic mono- or diselenide.

The composition of the invention, therefore, comprises three ingredients: a base oil, a salt of a phenol, and a selenium compound.

The base oil is preferably a mineral lubricating oil, such as a naphthenic, paraffinic or mixed base petroleum oil of lubricating viscosity, e. g., 150 to 3000 S. S. U. at 100° F. However, other oils, such as polypropylenes and polybutenes of lubricating viscosity, lubricating oils from synthetic petroleum such as derived from coal and oxides of carbon, and even non-hydrocarbon oils of lubricating viscosity such as polypropylene oxide, etc., may be used.

The salts of phenols or phenates used in accordance with the invention have the structure



in which A is an aromatic nucleus, M is a salt-forming atom or radical, and R is an ether-forming group attached to oxygen through carbon.

Preferably, the phenate is a polyvalent metal salt of a mono-ether of a dihydroxy benzene or a homologue of a dihydroxy benzene, and an aliphatic alcohol containing 5 to 30 carbon atoms; most advantageously the phenate is an

2

alkaline earth metal salt of a mono-ether of resorcinol or a homologue of resorcinol, in which the etherifying group is a C<sub>10</sub> to C<sub>30</sub> aliphatic radical.

Examples of suitable salts of phenols are as follows: lithium, sodium, potassium, calcium, strontium, barium, zinc and aluminum salts of ortho, meta- and para-pentoxy octoxy, decoxy, cetoxy, octadecoxy, eicosoxy, "paraffinoxy" and amylcyclohexoxy phenates. These particular examples have the generic formula



where R is an amyl, octyl, decyl, cetyl, octadecyl, eicosyl, paraffin or amylcyclohexyl radical (the "paraffin" radical being derived from paraffin wax by chlorination and condensation); M is lithium, sodium, potassium, calcium, strontium, barium, zinc or aluminum; the group —O—R is in the ortho, meta or para position with respect to the metaloxy group; and n is the valence of M. Basic and mixed salts may be used in place of normal salts, but the normal salts are preferred.

The selenium compounds of the compositions of the invention have the structure



wherein R<sub>1</sub> and R<sub>2</sub> are aliphatic radicals and m is 1 or 2. Thus, R<sub>1</sub> and R<sub>2</sub> may be alkyl, cycloaliphatic or aralkyl radicals. Preferably R<sub>1</sub> and R<sub>2</sub> are alkyl or aralkyl radicals each containing not less than 7 carbon atoms. Examples of suitable aliphatic selenium compounds are: dibutyl mono-selenide, di-amyl mono-selenide, di-octyl mono-selenide, di-octyl diselenide, octyl dodecyl mono-selenide, di-octadecyl mono-selenide, di-octadecyl diselenide, di—"paraffin" mono-selenide, di—"paraffin" diselenide, di-amylcyclohexyl mono-selenide, di-amylcyclohexyl diselenide and dibenzyl mono-selenide.

By the term "aliphatic radical" as used herein, without qualification, is meant radicals attached to selenium (in the case of the selenides) or to oxygen (in the case of the phenates) by a non-benzenoid carbon atom, and it includes, for example, alkyl, alkylenes, cycloalkyl and aralkyl radicals. By "selenide" as used herein, without qualifications as a mono- or diselenide, it is intended to include both the mono-selenides (R<sub>1</sub>—Se—R<sub>2</sub>) and diselenides (R<sub>1</sub>—Se<sub>2</sub>—R<sub>2</sub>).

To produce the finished oil of the invention

the phenate and the selenium compound may be incorporated in the base oil in proportions of about 0.1 to 2% each, by weight based on the finished oil. To produce concentrates or stock solutions, which are useful for later blending with more oil to produce the finished product, larger amounts, for example, 10 to 40%, of each of these additives may be incorporated in the oil.

The selenium compounds of the invention can be prepared by the methods described in Denison and Condit, United States Patent No. 2,398,414, issued April 16, 1946. A suitable mode of preparing the phenates of the invention is illustrated by the preparation of barium meta cetoxy phenate, as follows:

Equimolar proportions of resorcinol and cetyl

necessary to use a pure aliphatic chloride such as cetyl chloride, but crude mixtures such as chlorinated kerosene and chlorinated paraffin wax having an average molecular weight of 175 to 455, and preferably containing about one gram atom of chlorine per average gram molecular weight of mixture, may be used to alkylate the polyhydric phenol.

A further improvement in the preparation of the phenate additive of the invention is the employment of an excess of the polyhydric phenol. Such excess decreases the yield of di-ether and increases the yield of the desired mono-ether.

Oils of the invention were submitted to test as crankcase lubricants of gasoline engines with results as shown in the table:

Table

|                        | Base Oil                                        | Compounding                                                    | Piston Discoloration Number |         |
|------------------------|-------------------------------------------------|----------------------------------------------------------------|-----------------------------|---------|
|                        |                                                 |                                                                | 30 Hrs.                     | 60 Hrs. |
| LAUSON ENGINE TESTS    |                                                 |                                                                |                             |         |
| (1)                    | SAE 30 blend of paraffinic and naphthenic oils. | 16 mM./kg. Ba m-cetoxy phenate.....                            | 30                          | 75      |
| (2)                    | do.....                                         | 16 mM./kg. Ba m-cetoxy phenate+1% diisauryl monoselenide.      | 25                          | 45      |
| (3)                    | Pennsylvania base oil.....                      | Same as (2).....                                               | 20                          | 50      |
| WISCONSIN ENGINE TESTS |                                                 |                                                                |                             |         |
| (4)                    | SAE 50 blend of paraffinic and naphthenic oils. | Nil.....                                                       | 620                         | -----   |
| (5)                    | do.....                                         | Same as (2).....                                               | 105                         | 225     |
| (6)                    | do.....                                         | 16 mM./kg. Ba m-cetoxy phenate+1.54% di-paraffin monoselenide. | 20                          | 195     |
| (7)                    | do.....                                         | 16 mM./kg. Ba m-cetoxy phenate+0.625% di-benzyl monoselenide.  | 155                         | 245     |
| (8)                    | do.....                                         | Nil.....                                                       | 580                         | -----   |
| (9)                    | do.....                                         | Same as (2).....                                               | 80                          | 110     |
| (10)                   | do.....                                         | 16 mM./kg. Ba m-cetoxy phenate+0.8% di-octadecyl diselenide.   | 85                          | 100     |

chloride were dissolved in Cellosolve (trade-name of a product of Carbide and Carbon Chemicals Corp., being the mono-ethyl ether of ethylene glycol), and the solution was heated to reflux. To the refluxing mixture was slowly added solid potassium hydroxide and the refluxing was continued until all of the cetyl chloride had reacted. The Cellosolve was then removed by distillation and the reaction mixture was washed out of the flask with a petroleum thinner. Unreacted resorcinol and potassium chloride were washed out of the solution, first with water and then with 50% aqueous alcohol. The resorcinol monocetyl ether was recovered from the thinner solution as the potassium salt by washing with potassium hydroxide in 50% aqueous alcohol. The alkaline alcoholic solution was acidified and the liberated resorcinol monocetyl ether was extracted with petroleum ether and freed of petroleum ether by heating to 250° F. The normal barium salt was prepared by reacting the resorcinol monocetyl ether with barium oxide and the final product was recovered by extraction with lubricating oil to produce a concentrate.

The starting material for preparing the phenate additive need not be a pure polyhydric phenol, such as resorcinol, but may be a crude mixture of polyhydroxy benzenes or homologues of the same. In general, however, meta dihydroxy benzene and homologues of the same are preferred and where a crude mixture is used as the starting material, it is preferred to use a mixture in which the meta compounds predominate.

In alkylating the polyhydric phenol it is not

45 The amount of barium m-cetoxy phenate is stated in the table as 16 mM./kg., meaning 16 millimols of barium per kilogram of oil. That is, each oil containing the barium salt contained an amount equivalent to 16 millimols of barium per kilogram of oil.

50 Piston discoloration numbers as given in the table were determined by disassembling the test engines after 30 hours and again after 60 hours and inspecting the piston. A completely clean piston is rated as having a piston discoloration number (P. D. No.) of zero, a completely fouled piston, as having a P. D. No. of 300. Further refinements used in arriving at P. D. Nos. need not be given as the same method of rating was used in all cases.

55 The test engines were a Lauson single cylinder gasoline engine (oils Nos. (1) to (3)) operated at 460° F. jacket temperature and 220° F. oil sump temperature; a Wisconsin single cylinder gasoline engine (oils Nos. (4) to (7)) operated at 600° F. cylinder, 325° F. oil sump temperature; and a similar Wisconsin engine (oils Nos. (8) to (10)) operated at 600° F. cylinder, 220° F. oil sump temperatures.

60 The phenate and selenium additives of the invention may be used as the only compounding agents or they may be used in conjunction with other additives such as sulfonates (e. g., Ca mahogany sulfonate), phosphates (e. g., Ca cetyl phosphate) and thiophosphates (e. g., calcium and zinc di-cetylphenyl dithiophosphate and zinc di-methylcyclohexyl dithiophosphate); these additives being used in finished oils and in con-

centrates in proportions similar to those given above with regard to the phenates and selenium compounds of the invention.

We claim:

1. A composition of matter consisting essentially of a major proportion of a hydrocarbon oil of lubricating viscosity and about 0.1 to 2% by weight of each based on finished oil of a phenate having the structure  $R-O-A-O-M$ , in which A is an aromatic nucleus, M represents an alkaline earth metal, R is a hydrocarbon radical of 5-30 carbon atoms attached to the oxygen atom through a non-benzenoid carbon atom and the  $R-O$  group is in meta position in relation to the  $O-M$  group, and a selenium compound having the formula  $R_1-(Se)_m-R_2$ , wherein  $R_1$  and  $R_2$  are hydrocarbon radicals of at least 7 carbon atoms and attached to selenium by a non-benzenoid carbon atom, and  $m$  is 1 or 2.

2. The composition of claim 1 wherein the selenium compound is a dialkyl selenide containing not less than 8 carbon atoms in each alkyl group.

3. A mineral lubricating oil containing about 0.1 to 2% by weight each based on finished oil of an alkaline earth metal salt of a meta dihydric phenol having an alkyl radical of 5 to 30 carbon atoms substituted for the hydrogen of one of the hydroxyl radicals, and a selenium compound having the formula  $R_1-(Se)_m-R_2$ , wherein  $R_1$  and  $R_2$  are hydrocarbon radicals of at least 7 carbon atoms and attached to selenium by a non-benzenoid carbon atom, and  $m$  is 1 or 2.

4. The oil of claim 3, wherein said alkyl radical contains 10 to 30 carbon atoms.

5. A mineral lubricating oil containing about 0.1 to 2% by weight each based on finished oil of a salt of a phenol having the generic formula



wherein R is a hydrocarbon radical of 5-30 carbon atoms and is attached through a non-benzenoid carbon atom to the oxygen atom in meta position in relation to the metaloxy group, M is

an alkaline earth metal, and  $n$  is the valence of M and a dialkyl selenide containing not less than 8 carbon atoms in each alkyl radical.

6. The oil of claim 5, wherein said dihydric phenol is resorcinol.

7. A composition of matter consisting essentially of a major proportion of a hydrocarbon oil of lubricating viscosity and about 0.1 to 2% by weight of each based on finished oil of an alkaline earth metal phenate salt having a hydrocarbon ether ring substituent directly attached through the ether oxygen atom to the aromatic nucleus in the meta position in relation to the metaloxy group, said ether substituent containing 5-30 carbon atoms, and a selenium compound having the formula  $R_1-(Se)_m-R_2$ , wherein  $R_1$  and  $R_2$  are hydrocarbon radicals of at least 7 carbon atoms and attached to selenium by a non-benzenoid carbon atom, and  $m$  is 1 or 2.

8. A lubricant consisting essentially of a major proportion of a hydrocarbon oil of lubricating viscosity in about 0.1 to 2% by weight of each based on finished oil of metal salt of a meta dihydric phenol having substituted for the hydrogen of one of the hydroxy radicals of the parent dihydric phenol, a hydrocarbon radical of 5-30 carbon atoms directly attached to the oxygen through a non-benzenoid carbon atom, and a selenium compound having the formula



wherein  $R_1$  and  $R_2$  are hydrocarbon radicals of at least 7 carbon atoms and attached to selenium by a non-benzenoid carbon atom, and  $m$  is 1 or 2.

JAMES O. CLAYTON.  
WILLIAM H. ALDERSON.

#### REFERENCES CITED

The following references are of record in the 40 file of this patent:

#### UNITED STATES PATENTS

| Number    | Name     | Date          |
|-----------|----------|---------------|
| 2,197,833 | Reiff    | Apr. 23, 1940 |
| 2,344,988 | Kavanagh | Mar. 28, 1944 |
| 2,398,416 | Denison  | Apr. 16, 1946 |
| 2,402,448 | Richards | June 18, 1946 |